

## UNITED STATES PATENT OFFICE

2,222,487

## LUBRICANT

Johan C. D. Oosterhout and William S. Quimby,  
Port Arthur, Tex., assignors to The Texas Company,  
New York, N. Y., a corporation of Delaware

No. Drawing. Application September 29, 1937,  
Serial No. 166,326

3 Claims. (Cl. 252—51)

This invention relates to lubricants and has to do particularly with a light lubricating oil composition suitable for use as a household lubricant.

In compounding the lubricating oil composition, we use a light lubricating oil, preferably a highly refined paraffin base oil of about 60-150 Saybolt Universal viscosity at 100° F. and preferably about 100 viscosity.

With this oil we incorporate a small amount of a phosphatide, such as a material of the lecithin type; for example lecithin or cephalin. (Such phosphatide compounds occur naturally in substantial quantities in soybeans.) Commercial grades of lecithin known by the trade names "Lipoidol," "Coloidol H X" and "Coloidol B T" have been found satisfactory. The amount of phosphatide used ranges from  $\frac{1}{2}$  to 3%, and preferably about 1%.

Also we prefer to incorporate in the lubricating oil a small amount of a fatty oil, such as an animal oil, for example lard oil. The amount of fatty oil used may range from 2 to 10% and preferably about 5%.

In order to impart to the composition a pleasant odor, a small amount, for example about 0.06%, of an organic odorant or perfume, such as citronella may be added.

An improved composition which we have found to be particularly suitable comprises:

|                                     | Per cent |
|-------------------------------------|----------|
| Refined lubricating oil 100 Saybolt |          |
| Universal viscosity at 100° F.      | 94       |
| Prime lard oil                      | 5        |
| Lecithin                            | 1        |

The above product tested as follows:

|                                       |           |
|---------------------------------------|-----------|
| Gravity ° A. P. I.                    | 31.6      |
| Flash, Cleveland open cup ° F.        | 375       |
| Fire, Cleveland open cup ° F.         | 420       |
| Viscosity Saybolt Universal @ 100° F. | 101       |
| Color, 6" cell                        | 55        |
| Pour ° F.                             | 25        |
| Neutralization number                 | 0.08      |
| Iodine number                         | 15        |
| Saponification number                 | 9.1       |
| Sligh oxidation number                | 31.6      |
| Evaporation per cent                  | 8         |
| Rust proofing                         | Excellent |
| Stain test—discoloration              | None      |

The evaporation test was made according to the California State chemists method of evaporation in which one gram of oil is evaporated for a definite period at 212° F. from a mixture of the oil and 9 grams of sand.

The staining test was a modified method of the National Association of Hosiery and Underwear Manufacturers, in which the oil was poured on a cotton oily fabric and exposed to a weatherometer lamp for a definite period, washing the oily fabric with a soap or soda ash, dyeing the fabric and measuring the discoloration thereof.

The rust-proofing test consisted in dipping thin iron strips in oil, draining 18 to 24 hours at atmospheric temperature and then spraying with distilled water twice a day, at least 4 hours apart.

The lubricating oil composition herein described is a high grade household lubricant having improved properties with respect to stability, oiliness, staining and rust-proofing qualities.

Obviously many modifications and variations of the invention, as hereinbefore set forth, may be made without departing from the spirit and scope thereof and therefore only such limitations should be imposed as are indicated in the appended claims.

We claim:

1. A lubricant of the character described having superior rust-proofing properties consisting essentially of a light petroleum lubricating oil having a Saybolt viscosity at 100° F. of 60-150, about 2-10% of a fatty oil, and about 0.5-3.0% of a phosphatide.

2. A household lubricant having superior rust-proofing properties consisting essentially of a light petroleum lubricating oil having a Saybolt viscosity at 100° F. of 60-150, about 2-10% of lard oil, about 0.5-3% of a phosphatide, and a small amount of an organic odorant.

3. A household lubricant having superior rust-proofing properties consisting essentially of a light petroleum lubricating oil having a Saybolt viscosity at 100° F. of about 60-150, about 5% of lard oil, about 1% of lecithin, and a small amount of an organic odorant of the type of citronella.

JOHAN C. D. OOSTERHOUT.

WILLIAM S. QUIMBY.